

3,139,405

## EXTREME PRESSURE LUBRICANTS

Homer H. Farmer, Westport, and Harold F. Tompkins, Fairfield, Conn., assignors to R. T. Vanderbilt Company, Inc., New York, N.Y., a corporation of New York

No Drawing. Filed May 29, 1961, Ser. No. 113,150

6 Claims. (Cl. 252—33.6)

The present invention pertains to lubricants, and more particularly to extreme pressure lubricants.

With some types of gears, such as hypoid gears, and with heavily loaded bearings where both high pressure and high rubbing velocity occur, it is extremely difficult to maintain a thin film of lubricant between the bearing surfaces. When the film of lubricant ruptures, the mating high spots where metal-to-metal contact occurs are deformed and plow into each other resulting in localized welding. As the weld is sheared by the relative motion of the surfaces, particles of metal are removed. The contacting surfaces become rough and pitted and eventually fail by seizing or scoring.

The special types of lubricants developed for use under these conditions are known as "extreme pressure" or "E.P." lubricants. The E.P. lubricants are made by adding special E.P. agents to lubricating oils or to greases. Often other agents are also added, such as oiliness agents and anticorrosion agents.

Extreme pressure lubricants may prevent localized welding by reacting with the bearing surfaces. Some E.P. agents are thought to react with the surfaces to form low melting alloys, while others are thought to react to form easily sheared inorganic films.

It has been proposed heretofore to add some metallic salts of dialkyldithiocarbamic acids, e.g., tin diamyldithiocarbamate, lead diamyldithiocarbamate, and selenous diamyldithiocarbamate, as E.P. agents to mineral lubricating oils in order to form extreme pressure lubricants. While the extreme pressure properties of the lubricants are slightly improved by the use therein of these E.P. agents, nevertheless the lubricants so produced do not have the high load-carrying capacity or passing load now demanded by some present-day equipment subjected to unusually high pressures.

In accordance with the present invention there is provided an extreme pressure lubricating composition which has a load-carrying capacity or passing load which is exceedingly high and heretofore unobtainable by practical means. The extreme pressure lubricating composition of the invention comprises an oil or grease of mineral or synthetic origin, i.e., a lubricant, and a novel E.P. agent.

The lubricating oil base stock used in preparing the lubricant may be straight mineral lubricating oils or distillates, bright stock residua and the like. Synthetic lubricating oils, such as hydrogenated oils, glycol ethers, dibasic acid esters, and other polyester and polyether synthetic lubricating oils can be used. Mixtures of synthetic lubricating oils and petroleum base mineral oils can also be employed. The lubricating oil base stock will generally have a viscosity in the range of from about 40 to 150 seconds Saybolt viscosity at 210° F.

The novel E.P. agent or additive in the extreme pressure lubricating composition of the invention is antimonous diamyldithiocarbamate or antimonous dihexyldithiocarbamate. These materials can be readily prepared by reacting together antimony trioxide, carbon disulfide and commercial diamyl amine or dihexyl amine in accordance with the general process disclosed in U.S. Patent No. 2,492,314. The antimonous diamyldithiocarbamate or antimonous dihexyldithiocarbamate is present in the extreme pressure lubricating composition in an amount from

about 2.5% to about 5%, and preferably about 2.5%, based on the weight of the lubricating oil or grease, i.e., based on the weight of the lubricant.

The extreme pressure lubricating composition of the invention inhibits wear, scuffing and seizing of engaging movable parts subject to extreme pressures. It is characterized by having an exceptionally high Timken load-carrying capacity or passing load. Indeed, a Timken load-carrying capacity as high as 100 pounds can be obtained with a lubricant using the preferred amount of the antimonous diamyldithiocarbamate E.P. agent.

If desired, the extreme pressure lubricating composition can contain various optional components, such as oiliness agents, anticorrosion agents, pour depressants and other E.P. agents.

The extreme pressure lubricating composition of the invention can be used for a number of heavy duty purposes, such as a gear oil, cutting oil and metal working lubricant.

The amazingly high load-bearing capacity imparted to lubricants by the addition thereto of antimonous diamyldithiocarbamate or antimonous dihexyldithiocarbamate is indeed surprising and quite unexpected when it is considered that various other metallic salts of dialkyldithiocarbamic acids impart only moderate or low load-bearing capacities to lubricants. This is readily demonstrated by the comparative data set forth below in Table I.

The data in Table I were obtained in accordance with the following test procedure. To separate portions of a SAE 90 mineral lubricating oil having a viscosity of 87 seconds Saybolt viscosity at 210° F., 1030 seconds Saybolt viscosity at 100° F., and a viscosity index of 91 there were added various metallic salts of dialkyldithiocarbamic acids listed in Table I below to provide a dithiocarbamate content of 1%, 2%, 2.5%, 3%, 4%, 5%, and 10% based on the weight of the mineral lubricating oil. The lubricating compositions so produced were subjected to the Timken load-bearing test in the Timken Lubricant Tester in which a hardened steel ring rotating at 800 r.p.m. was flooded by the test lubricating composition at 100° F. while a hardened steel block was pressed against it by a system of weights and levers. The highest weight which did not produce scoring of the block in ten minutes running time was recorded as the passing load or O.K. load, which is a recognized measure of the load-carrying capacity of a lubricant. The values obtained in accordance with this standard test are set forth in Table I below.

Table I

| Percent by Weight of Additive in SAE 90 Mineral Lubricating Oil |                                             | 1            | 2  | 2.5 | 3  | 4  | 5                      | 10                     |
|-----------------------------------------------------------------|---------------------------------------------|--------------|----|-----|----|----|------------------------|------------------------|
| Additive                                                        |                                             | Passing Load |    |     |    |    |                        |                        |
| 55                                                              | Antimonous diamyldithiocarbamate            | 20           | 40 | 100 | 90 | 90 | 80                     | 70                     |
|                                                                 | Antimonous dihexyldithiocarbamate           | 20           | 50 | 90  | —  | —  | 85                     | —                      |
|                                                                 | Antimonous dibutylidithiocarbamate          | 20           | 50 | 80  | 80 | —  | —                      | —                      |
|                                                                 | Antimonous di-2-ethylhexylidithiocarbamate  | —            | —  | —   | 25 | —  | —                      | —                      |
|                                                                 | Antimonous didecyldithiocarbamate           | —            | —  | —   | 25 | —  | —                      | —                      |
|                                                                 | Lead diamyldithiocarbamate                  | 55           | 65 | 60  | 30 | 30 | 30                     | 20                     |
|                                                                 | Arsenous diamyldithiocarbamate              | 20           | 30 | 30  | —  | —  | Insoluble <sup>2</sup> | —                      |
| 60                                                              | Selenous diamyldithiocarbamate <sup>1</sup> | 30           | 50 | 50  | 40 | 30 | 30                     | —                      |
|                                                                 | Bismuthous diamyldithiocarbamate            | 30           | 65 | 50  | 40 | 40 | 30                     | 30                     |
|                                                                 | Zinc diamyldithiocarbamate                  | 20           | 30 | 40  | 40 | 40 | 40                     | 30                     |
|                                                                 | Cadmium diamyldithiocarbamate               | 30           | —  | 30  | 50 | 50 | 40                     | 40                     |
|                                                                 | Stannic diamyldithiocarbamate               | 20           | 30 | 60  | 40 | —  | —                      | Insoluble <sup>2</sup> |
|                                                                 | Bismuthous dibutylidithiocarbamate          | —            | —  | —   | —  | —  | —                      | —                      |
| 65                                                              | Nickelous dibutylidithiocarbamate           | —            | —  | —   | —  | —  | —                      | Insoluble <sup>2</sup> |

<sup>1</sup> Impure selenous diamyldithiocarbamate containing tetraamyl thium disulfide.

<sup>2</sup> Additive crystallized out and clogged filter of Timken Lubricant Tester. Test discontinued.

The data set forth in Table I above establish that the extreme pressure lubricating compositions of the invention containing from about 2.5% to about 5%, of anti-

monous diamyldithiocarbamate or antimonous dihexylthiocarbamate based on the weight of the mineral lubricating oil have an exceptionally high Timken load-carrying capacity, even as high as 100 pounds, which values were heretofore considered to be unobtainable by practical means. None of the comparative lubricants containing analogous or homologous dithiocarbamates could approach the remarkable load-carrying capacity of the extreme pressure lubricating compositions of the invention. Indeed, several of the comparative dithiocarbamate salts were insoluble in the mineral lubricating oil and accordingly did not impart any extreme pressure properties thereto.

Although the comparative test results given above were obtained with a Timken Lubricant Tester, corroborating data were obtained using the Shell 4-Ball and Falex testing machines.

The Timken load-bearing capacity of a typical grease, namely a lithium 12-hydroxystearate grease, to which antimonous diamyldithiocarbamate had been added at 1%, 2%, 3% and 4% by weight of the grease is presented in Table II below.

Table II

| Percent by Weight of Additive in a lithium 12-hydroxystearate grease | 1            | 3  | 3  | 4  |
|----------------------------------------------------------------------|--------------|----|----|----|
| Additive                                                             | Passing Load |    |    |    |
| Antimonous diamyldithiocarbamate                                     | 10           | 35 | 80 | 80 |

It will be appreciated that various modifications and changes in addition to those set forth above may be made in the compositions of the invention without departing from the spirit thereof, and accordingly the invention is to be limited only within the scope of the appended claims.

What is claimed is:

1. An extreme pressure lubricating composition for inhibiting wear, scuffing and seizure of engaging movable parts subject to extreme pressures consisting essentially of a lubricant selected from the group consisting of fluid lubricants and greases, and from about 2.5% to about 5% based on the weight of the lubricant of an antimonous dialkyldithiocarbamate extreme pressure additive selected

from the group consisting of antimonous diamyldithiocarbamate and antimonous dihexylthiocarbamate.

2. An extreme pressure lubricating composition for inhibiting wear, scuffing and seizure of engaging movable parts subject to extreme pressures consisting essentially of a lubricating grease and from about 2.5% to about 5% based on the weight of the lubricating grease of an antimonous dialkyldithiocarbamate extreme pressure additive selected from the group consisting of antimonous diamyldithiocarbamate and antimonous dihexylthiocarbamate.

3. An extreme pressure lubricating composition for inhibiting wear, scuffing and seizure of engaging movable parts subject to extreme pressures consisting essentially of a lubricating oil and from about 2.5% to about 5% based on the weight of the lubricating oil of an antimonous dialkyldithiocarbamate extreme pressure additive selected from the group consisting of antimonous diamyldithiocarbamate and antimonous dihexylthiocarbamate.

4. An extreme pressure lubricating composition for inhibiting wear, scuffing and seizure of engaging movable parts subject to extreme pressures consisting essentially of a mineral lubricating oil and from about 2.5% to about 5% based on the weight of the mineral lubricating oil of antimonous diamyldithiocarbamate as an extreme pressure additive.

5. An extreme pressure lubricating composition for inhibiting wear, scuffing and seizure of engaging movable parts subject to extreme pressures consisting essentially of a mineral lubricating oil and from about 2.5% to about 5% based on the weight of the mineral lubricating oil of antimonous dihexylthiocarbamate as an extreme pressure additive.

6. An extreme pressure lubricating composition for inhibiting wear, scuffing and seizure of engaging movable parts subject to extreme pressures consisting essentially of a mineral lubricating oil and about 2.5% based on the weight of the mineral lubricating oil of antimonous diamyldithiocarbamate as an extreme pressure additive.

## 40 References Cited in the file of this patent

## UNITED STATES PATENTS

2,716,089 Cypers et al. ----- Aug. 23, 1955

## FOREIGN PATENTS

45 211,212 Australia ----- May 17, 1956

506,167 Canada ----- Sept. 28, 1954

UNITED STATES PATENT OFFICE  
CERTIFICATE OF CORRECTION

Patent No. 3,139,405

June 30, 1964

Homer H. Farmer et al.

It is hereby certified that error appears in the above numbered patent requiring correction and that the said Letters Patent should read as corrected below.

Column 2, Table I, first column, line 15 thereof, for "Cadmium" read -- Cadmium --; column 3, Table II, line 2 thereof, for "1 3 3 4" read -- 1 2 3 4 --; column 4, line 42, for "Cypers et al." read -- Cyphers et al. --.

Signed and sealed this 10th day of November 1964.

(SEAL)

Attest:

ERNEST W. SWIDER  
Attesting Officer

EDWARD J. BRENNER  
Commissioner of Patents